

# UNITED STATES PATENT OFFICE.

WILLIAM FEENIE, OF BUHL, MINNESOTA, AND WILLIAM W. RHODES, OF WILMINGTON, DELAWARE, ASSIGNORS TO E. I. DU PONT DE NEMOURS & COMPANY, OF WILMINGTON, DELAWARE, A CORPORATION OF DELAWARE.

## PROCESS OF REMOVING SCALE OXID FROM THE SURFACE OF IRON AND STEEL.

1,326,585.

Specification of Letters Patent. Patented Dec. 30, 1919.

No Drawing.

Application filed April 3, 1919. Serial No. 287,361.

*To all whom it may concern:*

Be it known that we, WILLIAM FEENIE and WILLIAM W. RHODES, citizens of the United States, and residents of Buhl, county 5 of St. Louis, State of Minnesota, and of Wilmington, county of New Castle, and State of Delaware, respectively, have invented certain new and useful Processes of Removing Scale Oxid from the Surface of 10 Iron and Steel, of which the following is a specification.

This invention relates to a process of removing the metal oxid which is usually present as a scale on the surface of rolled or 15 hammered iron or steel, and on the surface of alloy steels; and the invention pertains especially to the dissolving of such scale with the aid of a solution of a metal bisulfate.

20 A widely used process for removing scale from iron and steel consisted in subjecting the iron or steel stock to the action of a water solution containing sodium bisulfate and also, in some cases, stannous sulfate.

25 Other methods of pickling iron or steel usually involved the use of an acid such as sulfuric acid. Although sulfuric acid was not as desirable a pickling agent as sodium bisulfate because of its dissolving action on 30 the metal itself, it was nevertheless frequently used instead of sodium bisulfate on account of the lower cost of the process as compared with the process using sodium bisulfate. In working with the latter it

35 was found that the solution became inactive as far as its ability to remove scale was concerned after a certain percentage of the bisulfate had been used up, but while a considerable proportion of bisulfate remained unchanged. Since it seemed impracticable to render all of the bisulfate available for

40 pickling, it was looked upon unfavorably from a cost standpoint in comparison with sulfuric acid, even though the pickled product showed less pitting and was better pickled than the steel stock pickled with a solution of sulfuric acid. Only manufacturers who desired especially fine pickling regardless of cost could afford to use bisulfate.

45 The principal object of our invention is to provide a process of removing scale oxid with a solution of sodium bisulfate whereby

a much larger proportion of the bisulfate in solution is rendered available than was the case in the old process.

55 Another object of our invention is to so modify the ordinary bisulfate pickling solution that it may be successfully used to remove the scale from alloy steels, such as nickel, chrome and vanadium steels.

60 The pickling action may be explained as follows:

The sodium acid sulfate attacks the ferrous oxid according to the following equation:



65 For every molecule of ferrous oxid dissolved, two molecules of sodium acid sulfate are used up in producing one molecule each of sodium sulfate, ferrous sulfate and water.

70 In pickling with niter cake, which is commonly used for this purpose, there is present about 22% sodium sulfate in the cake, so that the fresh bath contains sodium sulfate as such.

75 In the fresh bath sodium acid sulfate is highly dissociated, but as the amount of sodium acid sulfate diminishes due to its conversion to sodium sulfate and ferrous sulfate and the concentration of the sodium sulfate and ferrous sulfate increases, the dissociation of sodium acid sulfate diminishes until it reaches practically zero, for there is no perceptible action on the iron or steel stock.

80 A pickling bath of niter cake which has become inactive may be made active again in some degree by the addition of water, but the concentration of the sodium bisulfate is thereby diminished and the resulting speed of pickling is too slow for commercial practice.

85 We have discovered that the activity of a bisulfate solution which has been used for pickling until it has become almost inactive, may be greatly increased by decreasing the ratio of the normal sulfates to the bisulfates, and especially by removing sodium sulfate. 100 The temperature of the bath during pickling is between 100 and 200° F., and preferably about 140° F. We have found that a convenient method for decreasing the ratio of normal sulfates to bisulfates comprises reducing the temperature by about 50 or 105

60° F. When the solution is cooled to this extent, for example from 140° F. to 85° F., a large proportion of the sodium sulfate and a smaller proportion of the ferrous sulfate 5 contained in solution will crystallize and become segregated in a watery layer near the bottom of the tank, whereas all of the bisulfate present will remain in solution. The layer containing crystallized sodium sulfate 10 is then separated from the supernatant liquid; the latter will be found to have regained by this treatment an activity or speed approaching that of a fresh solution containing the same amount of sodium bisulfate. The expression "speed of pickling" 15 is used to denote a comparison of the elapsed time the steel or iron stock requires to pickle compared with the standard elapsed time for pickling in a fresh solution.

20 The following specific example will illustrate the practical working of our new process. The practice followed in this example is to produce maximum efficiency with a very fair rate of speed, but not maximum 25 speed because with maximum speed the efficiency is somewhat sacrificed.

We shall take for example as stock to be pickled iron wire varying from 10 gage B. & S. to  $\frac{3}{8}$ " rods.

30 A pickling tank of approximately 160 cubic feet capacity is used so that when filled to the working level it will contain 1000 gallons of water. The tank is filled with 1000 gallons of water and 1500 lbs. of niter cake 35 added, and the niter cake dissolved. The temperature of the solution is brought up to approximately 140° F. and maintained at that temperature as nearly as possible. There is now added a rack of the stock containing a net weight of 2400 lbs. of wire and this stock is allowed to pickle one-half hour, when the scale and oxid will have been removed. This rack of stock is now removed and another added and allowed to 40 pickle for one-half hour; this procedure is continued until a total of four racks or 9600 lbs. of wire have been pickled. If, at this point, no further niter cake were added to the solution, the speed of pickling would 45 rapidly diminish; 300 lbs. of niter cake is added and allowed to dissolve. Two more racks are then pickled, allowing each to remain submerged one-half hour. The total quantity now pickled is 14,400 lbs. of wire.

50 55 300 lbs. of niter cake are again added and two more racks are pickled so that the total becomes 19,200 lbs. of wire pickled.

Three hundred more pounds of cake are then added and two more racks pickled.

60 There has now been pickled 24,000 lbs. of wire and a total of 2400 lbs. of niter cake has been added to the bath.

The bath is now near its saturation point for salts, viz.,  $2\frac{1}{2}$  lbs. per gallon, and if the 65 pickling were continued it would soon di-

minish in speed and become inactive, although there is still sodium acid sulfate present.

The tank is now allowed to cool, e. g., to 90° F. The saturation of the tank is high 70 in respect to all the salts present, viz., sodium sulfate, ferrous sulfate and sodium acid sulfate. The sodium acid sulfate is ten times more soluble than sodium sulfate and one and one-half times more soluble than 75 ferrous sulfate. When this quiescent saturated solution cools the sodium sulfate crystallizes and separates as a watery layer near the bottom of the tank and mixed with it is usually a certain amount of crystallized ferrous sulfate. The mechanically removed sludge is also on the bottom of the tank.

25% of the cubical contents of the tank lying near the bottom is then slowly drained off through a suitable outlet. This removes 85 the mechanical sludge, a great portion of the sodium sulfate and some of the ferrous sulfate.

The tank is now made up to its original level with water and 25% of the original 90 charge of niter cake added, viz., 375 lbs. The temperature is now raised to 140° F., and exactly the same pickling procedure down to the draw off as outlined above is followed, so that 48,000 lbs. of wire is completed as a total to this point.

Another draw off is resorted to and the schedule repeated and the total wire pickled becomes 72,000 lbs. Still another draw off may be made and the schedule again repeated until a grand total of 96,000 lbs. of wire has been pickled.

As stated above, it is not possible to eliminate the ferrous sulfate entirely by the draw off method, and at this point the ferrous 105 sulfate becomes very concentrated and the solution has gradually assumed a greenish appearance. Nothing can now be done to maintain its speed and the tank is consequently emptied of its entire contents.

The amount of steel pickled per unit of acidity by this new bisulfate process is greater than for a solution of sulfuric acid, due to the fact that we have established a procedure wherein the acid content of the 115 sodium bisulfate or niter cake has been made effective and also due to the fact that sodium bisulfate attacks only the oxid and has little action on the iron after it becomes bared of its oxid coating.

The greatly increased efficiency of this new process over the old process is easily seen, for in the old process to maintain fair speed it was only possible to pickle ten pounds of wire per pound of niter cake used, whereas in the present process 15.4 pounds of wire may be pickled per pound of niter cake used; i. e., a 50% greater yield of pickled product from the same quantity of sodium bisulfate.

We claim:

1. The process of removing scale oxid from iron and steels which comprises subjecting the scale-coated metal to the action 5 of an unsaturated sodium bisulfate solution, maintained at a temperature of from 100° to 200° F., thereby incidentally forming normal salts, adding further amounts of sodium bisulfate to said solution to enable said solution 10 to exert a solvent action on further quantities of scale-coated metal, subjecting further quantities of metal to the resulting solution, continuing to make such additions until said solution becomes saturated with 15 salts and no longer exerts a vigorous solvent action on scale, and then decreasing the ratio of the normal salts to the sodium bisulfate to restore the scale-dissolving activity of the bisulfate solution.
2. The process of removing scale oxid 20 from iron and steels which comprises subjecting the scale-coated metal to the action of an unsaturated sodium bisulfate solution, maintained at a temperature of from 25 100° to 200° F., thereby incidentally forming normal salts, adding further amounts of sodium bisulfate to said solution to enable said solution to exert a solvent action on further quantities of scale-coated metal, 30 subjecting further quantities of metal to the resulting solution, continuing to make such additions until said solution becomes saturated with salts and no longer exerts a vigorous solvent action on scale, then lowering 35 the temperature of the solution to precipitate at least part of the relatively insoluble normal salts contained therein, separating the precipitate from the remaining bisulfate solution, and subjecting further 40 quantities of scale-coated metal to the action of said remaining bisulfate solution.
3. The process of removing scale oxid 45 from iron and steels which comprises subjecting the scale-coated metal to the action of an unsaturated sodium bisulfate solution, maintained at a temperature of about 140° F., thereby incidentally forming normal salts, adding further amounts of sodium bisulfate to said solution to enable said solution 50 to exert a solvent action on further quantities of scale-coated metal, subjecting

further quantities of metal to the resulting solution, continuing to make such additions until said solution becomes saturated with salts and no longer exerts a vigorous solvent action on scale, then lowering the temperature of the solution to precipitate at least part of the sodium sulfate contained therein, separating the precipitate from the remaining solution, and subjecting further quantities of scale-coated metal to the action of said remaining solution at an elevated temperature.

4. The process of removing scale oxid from iron and steels which comprises subjecting the scale-coated metal to the action of a saturated solution of sodium bisulfate at an elevated temperature until the normal sodium sulfate in solution has accumulated to such an extent as to effectually weaken the solvent action of the remaining bisulfate, then removing at least a substantial part of said normal sodium sulfate which is in solution to render said solution unsaturated with respect to said normal sulfate at said elevated temperature, and subjecting further quantities of scale-coated metal to the action of the resulting bisulfate-containing solution.

5. In the process of removing scale-oxid from iron and steels the step of restoring the scale-dissolving action of a sodium bisulfate solution which has become inactive which comprises so decreasing the ratio of normal sulfate, which is present in said solution, to the bisulfate as to render said solution unsaturated at normal working temperature with respect to sodium sulfate.

6. In the process of removing scale-oxid from iron and steels the steps of restoring the scale-dissolving action of a sodium bisulfate solution which has become inactive which comprise so cooling the solution as to precipitate normal sodium sulfate while avoiding precipitation of substantial proportions of sodium bisulfate, and separating the precipitate from the remaining solution.

In testimony whereof we affix our signatures.

WILLIAM FEENIE.  
WILLIAM W. RHODES.